

## UNITED STATES PATENT OFFICE

2,386,890

## WORK HARDENING ALLOY STEEL

Albert Paul Gagnebin, Red Bank, N. J., assignor  
to The International Nickel Company, Inc.,  
New York, N. Y., a corporation of Delaware

No Drawing. Application April 14, 1943,  
Serial No. 483,049

7 Claims. (Cl. 75—128)

The present invention relates to work hardening alloy steels.

It has been proposed to use Hadfield's manganese steel containing about 10% to 14% manganese for many applications where wear resistance and abrasion resistance were desired, for example, in digging and crushing machinery requiring toughness and abrasion resistance. However, Hadfield's austenitic manganese steel suffered from several shortcomings. It required a toughening heat treatment, i. e., the steel had to be heat treated in order to prevent brittleness. The steel developed useful properties only after water quenching from about 1900° F. This drastic treatment often caused cracks and usually caused distortion requiring subsequent straightening. Moreover, its application was restricted to section sizes under about 5 inches thick because the quenching stresses developed in the heavier sections promoted internal cracks leading to early failure. In addition, it could be produced only in certain limited types of furnace equipment. It could not be produced in the acid electric furnace, which is in common use in jobbing foundries, but was produced only in a basic electric furnace or by mixing molten steel and separately melted ferro-manganese. Furthermore, it required the use of large quantities of the strategically necessary manganese. Although many attempts were made to remedy the aforementioned and other shortcomings, none, as far as I am aware, was entirely successful when carried into practice commercially.

I have discovered that the prior art shortcomings can be avoided and that new and unexpected results can be obtained by using a special combination of elements in controlled proportions.

It is an object of the present invention to provide a cast steel alloy which hardens rapidly when bruised or deformed.

It is another object of the invention to provide an alloy steel which is tough in the as cast condition and which can be hardened to a high level of hardness by cold deformation.

It is a further object of the invention to provide a cast alloy steel which is tough and wear resistant.

It is also an object of the invention to provide a cast alloy steel of the work hardening type which does not require a heat treatment to prevent brittleness.

It is still another object of the invention to provide an alloy steel of the work hardening type which does not require the large amounts of manganese required heretofore.

The invention also provides an alloy steel of the work hardening type which can be produced with furnace equipment not suited for the production of Hadfield's manganese steel, e. g., with an acid lined furnace.

Other objects and advantages of the invention will become apparent from the following description.

Generally speaking, the present invention provides an alloy steel which is tough in the as cast condition, which work hardens rapidly, and which can be produced in the acid electric furnace, in addition to other furnace equipment. The iron base alloy steels provided by the present invention contain about 3% to 10% nickel, about 1.5% to 3% or 3.5% chromium, about 2% to 6% manganese, and about 0.8% to 1.7% or 1.8% carbon. A more preferred range is about 4% to 8% nickel, about 1.7% to 2.75% or 3% chromium, about 3% to 5.5% manganese, and about 1% to 1.5% carbon. In addition, the alloy steels of the present invention may contain small amounts of incidental or minor constituents and impurities added for known purposes or present as a result of good steel making practices, e. g., special deoxidizers, silicon, phosphorus, sulphur, etc. Thus, the steels normally will contain about 0.1% up to 1%, or even more, of silicon, e. g., about 0.4% to 0.5%. It is to be understood that when the term "balance substantially all iron" is used herein, it is not desired to exclude incidental or minor constituents or impurities which may be present in such amounts as occur in commercial products or in amounts not adversely affecting the desired properties of the alloy steel.

In carrying the invention into practice, the nickel, chromium and manganese contents must be so correlated that the minimum amounts of all the elements are not used in any one composition. Similarly, the maximum amounts of all the elements should not be used in one composition. If the minimum amounts of nickel, chromium and manganese are used, toughness in the as cast condition is sacrificed; whereas, if the maximum amount of each of these elements is used, the rapid work hardening properties are deleteriously affected. I have found that the sum of the nickel, chromium and manganese must be maintained within a certain range to obtain the desired results. The correlation of nickel, chromium and manganese has been termed herein the "alloy factor" and is defined as the sum of the nickel content, plus the chromium content, plus twice the manganese content. The alloy factor should be at least about 11%, preferably 13%, and should not exceed about 20% or 21%, preferably 18%.

The alloy steels provided by the present invention do not require a heat treatment and thus permit a great latitude in the shape and design of castings capable of successful production. For example, light and heavy sections can be combined in a single casting, which is not possible with Hadfield's manganese steel because the high quenching stresses developed by the different

cooling rates of thick and thin sections cause cracking. The absence of heat treatment and attendant distortion also means that castings of the new alloy steel will fit properly in the units for which they are intended. Hadfield's manganese steel cannot be produced in an acid lined furnace because the manganese in the steel oxidizes rapidly and reacts with the lining of the furnace causing a rapid erosion of the refractory and large losses in the manganese content. Since the new alloy contains less than about 6% manganese, preferably about 4.5% manganese, and one-half of this quantity can be melted in the furnace and the other half added to the ladle, its production in acid electric furnaces offers little difficulty.

In actual practice, the alloy steels of the present invention preferably contain at least 5% nickel, e. g., about 5.5% to 7% nickel, at least 2% chromium, e. g., about 2% to 2.5% chromium, at least 3.5% manganese, e. g., about 4% to 5% manganese, and at least 1.1% carbon, e. g., about 1.1% to 1.4% carbon.

The composition of the alloy steels provided by the present invention is so controlled that the cast steel has a microstructure containing substantial amounts of austenite which is sufficiently unstable to transform when bruised or subjected to cold deformation. The as cast microstructure may also contain some martensite. The greater the proportion of not too stable austenite, the tougher is the steel in the as cast condition. In general, the steel will be slightly magnetic.

In the steels of the present invention, chromium, within the ranges set forth hereinabove, is essential to achieve the desired results. I have made the surprising discovery that chromium reduces the carbide network and appears essential to secure toughness in the as cast condition in an alloy steel which will rapidly work harden. Likewise, a sufficiently high carbon content is essential to obtain desired results. In general, the ranges set forth are critical and if the alloy content falls below the minimum or maximum set forth, the desired combination of toughness and rapid work hardening properties is no longer obtained.

Illustrative examples of steels having compositions contemplated by the present invention are set forth in the table.

Table

| Steel No. | Per cent Ni | Per cent Mn | Per cent Cr | Per cent Si | Per cent C |
|-----------|-------------|-------------|-------------|-------------|------------|
| 1.....    | 6.2         | 4.5         | 2.3         | 0.26        | 1.3        |
| 2.....    | 5.9         | 3.7         | 2.1         | 0.51        | 1.1        |
| 3.....    | 6           | 5           | 2           | 0.5         | 1.2        |

The as cast toughness of these steels is very high in both light and heavy sections. The toughness can be improved further by chill casting which refines the grain and increases the austenitic stability. Chilling the working face on particularly severe applications is advantageous. The toughness can also be improved further by water quenching from a high temperature. The steels of the present invention work harden as well as austenitic manganese steel. Thus, Steel No. 1 has an as cast hardness of about 10 to 14 Rockwell "C" which increased to about 43 Rockwell "C" after a given amount of

5 cold deformation. An austenitic manganese steel containing 14.5% manganese and 1.3% carbon, and having an as cast hardness of about 10 Rockwell "C," had a hardness of about 38 Rockwell "C" after being subjected to about the same amount of cold deformation as was Steel No. 1. With more severe cold deformation the steels of the present invention, e. g., Steel No. 1, develop hardnesses as high as 50 Rockwell "C" or more.

10 The steels provided by the present invention are adaptable in cast or wrought form for use in digging, crushing and grinding applications requiring toughness and abrasion resistance. Examples of suitable applications include ball mill liners, jaw plates in crushers, rolls, etc.

15 Although the present invention has been described in conjunction with preferred embodiments, it is to be understood that modifications and variations may be resorted to without departing from the spirit and scope of the invention, as those skilled in the art will readily understand. Such variations and modifications are considered to be within the purview and scope of the invention and the appended claims.

I claim:

20 1. An alloy steel containing about 5% to 7% nickel, about 2% to 2.5% chromium, about 3.5% to 5% manganese, about 1.1% to 1.4% carbon, and the balance substantially all iron.

25 2. An alloy steel containing about 4% to 8% nickel, about 1.7% to 3% chromium, about 3% to 5.5% manganese, the sum of the nickel content, the chromium content, and twice the manganese content being at least about 13% and not more than about 18%, about 1% to 1.5% carbon, and the balance substantially all iron.

30 3. An alloy steel containing about 3% to 10% nickel, about 1.5% to 3.5% chromium, about 2% to 6% manganese, the sum of the nickel content, the chromium content and twice the manganese content being at least about 13% and not more than about 18%, about 0.8% to 1.8% carbon, and the balance substantially all iron.

35 4. An alloy steel containing about 3% to 10% nickel, about 1.5% to 3.5% chromium, about 2% to 6% manganese, the sum of the nickel content, the chromium content and twice the manganese content being at least about 11% and not more than about 21%, about 0.8% to 1.8% carbon, and the balance substantially all iron.

40 5. As an article of manufacture, a casting made of an alloy steel containing about 5% to 7% nickel, about 2% to 2.5% chromium, about 3.5% to 5% manganese, about 1.1% to 1.4% carbon, and the balance substantially all iron.

45 6. As an article of manufacture, a casting made of an alloy steel containing about 4% to 8% nickel, about 1.7% to 3% chromium, about 3% to 5.5% manganese, the sum of the nickel content, the chromium content, and twice the manganese content being at least about 13% and not more than about 18%, about 1% to 1.5% carbon, and the balance substantially all iron.

50 7. As an article of manufacture, a casting made of an alloy steel containing about 3% to 10% nickel, about 1.5% to 3.5% chromium, about 2% to 6% manganese, the sum of the nickel content, the chromium content and twice the manganese content being at least about 11% and not more than about 21%, about 0.8% to 1.8% carbon, and the balance substantially all iron.

55 ALBERT PAUL GAGNEBIN.